

Feb. 27, 1923.

1,446,678

C. T. WILKS

METHOD OF MAKING CASTINGS OF COMPOSITE METALS

Filed Dec. 11, 1920



Inventor:  
Charles T. Wilks,  
by Ruppel & Uppland  
his Attorney

Patented Feb. 27, 1923.

1,446,678

# UNITED STATES PATENT OFFICE.

CHARLES T. WILKS, OF CLINTON, MISSOURI.

## METHOD OF MAKING CASTINGS OF COMPOSITE METALS.

Application filed December 11, 1920. Serial No. 429,864.

To all whom it may concern:

Be it known that I, CHARLES T. WILKS, a citizen of the United States, residing at Clinton, Henry County, Missouri, have invented a new and useful Method of Making Castings of Composite Metals, of which the following is a specification.

This invention relates to improvements in method of making castings of composite metal.

Heretofore in practice attempts have been made to fuse bronze with iron, semi-steel or steel to make a composite casting having a section of the bronze integrally united with a section of the iron, semi-steel or steel. Such efforts have been unsuccessful in forming castings having a perfect union between the two metals. By continued experiment I have developed a method whereby a casting may be formed having a layer or section of bronze integrally united with a layer or section of iron, semi-steel or steel.

The object of this invention, therefore, is the production of a method for forming composite castings from bronze and iron, semi-steel or steel integrally united.

The invention may be better understood by the following description taken in connection with the drawing, which is submitted for illustrative purposes only, which drawing discloses a vertical section through a mold utilized in the practice of the method or process.

The mold in which the castings are formed is of the usual type comprising a drag 1 and a cope 2. A mold cavity 3 is formed in the sand 4 carried by the drag. Running through the sand body 5 of the cope and into the mold cavity, preferably at opposite ends, are duplicate gate or riser passages 6 and 7. The passages 6 and 7 are arranged to enter the mold cavity at a level corresponding to the upper surface of the layer of bronze.

The method in which the casting is poured consists in providing a molten mixture including copper, lead and tin mixed substantially in the proportion of eighty, ten and ten. The molten mixture is poured into either of the openings 6 and 7, the mold being filled to the level of the inlet of the pouring passage. The quantity of molten metal required to fill the mold cavity to the pre-determined level is calculated in advance, so that the pouring ladle contains just sufficient metal to raise the level in the

mold cavity to the throat of the pouring cavity.

After the bronze or copper alloy has been poured a sufficient interval of time is allowed for it to partially solidify or come to a semi-molten state in the mold. The iron, semi-steel or steel mixture is then poured from the other pouring passage into the mold, the first pouring passage constituting a riser passage for the metal.

It has been found by experiment that in order to accomplish satisfactory results it is necessary that the iron, semi-steel or steel shall include at least one per cent manganese, and also that no zinc shall be included in the copper alloy.

The casting poured as above described, results in a perfect union along a substantially well defined line which, however, is somewhat irregular due to the irregular upper surface of the first pouring of the metal. It is important that the first layer be allowed to partially solidify in order to prevent it from becoming mixed with the second layer.

The general theory of the process is that the bronze mixture having a lower melting point than the iron and being allowed to cool will maintain its conformation throughout the body when the iron, semi-steel or steel mixture is poured upon it, and that the higher melting point of the molten iron, semi-steel or steel will sufficiently raise the temperature of the surface of the lower layer to cause it to intermix for a sufficient depth with the second pouring, so that the two will unite forming a substantially perfect union between the two layers.

The sequence in which the layer of molten iron, semi-steel or steel and the layer of the bronze mixture is poured may be reversed, although it is preferable that the bronze mixture be poured first. An interval of time is allowed between the pouring of the layer of iron, semi-steel or steel to allow the same to cool slightly before the bronze is poured so that the bronze will not go through the first layer.

I claim:

1. The method of forming composite castings composed of a copper alloy free from zinc; and iron, semi-steel or steel, which consists in pouring a molten copper alloy into a mold to form a stratum in the bottom of the mold; permitting said stratum to come to a semi-molten state; and then pouring into

the mold onto the semi-molten stratum a quantity of molten iron, semi-steel or steel to increase the heat of the contiguous copper alloy and to form undulations in the same 5 to form a stratum having a thickness from the top of the first stratum to the top wall of the mold.

2. The method of forming a composite casting, composed of a copper alloy free 10 from zinc; and iron, semi-steel or steel, which consists in pouring a quantity of the molten copper alloy free from zinc and including copper, lead and tin, into a mold to form a stratum in the bottom of the mold; permitting 15 said stratum to come to a semi-molten state; and then pouring into the mould onto the first stratum a quantity of molten iron, semi-steel or steel, including at least one per cent manganese, to increase the heat of the 20 contiguous copper alloy and to form undulations in the same to form a stratum having a thickness from the top of the first stratum to the opposite wall of the mold.

3. The method of forming a composite 25 casting composed of a copper alloy free from zinc; and iron, semi-steel or steel, which consists in pouring the molten copper alloy free from zinc, and composed of copper, lead and

tin mixed substantially in the proportions of eighty per cent copper, ten per cent lead, 30 and ten per cent tin, into a mold to form a stratum in the bottom of the mold; causing said stratum to come to a semi-molten state; and then pouring into the mold onto the first stratum a quantity of molten iron, semi-steel or steel including at least one per cent manganese, to increase the heat of the contiguous copper alloy and to form undulations in the same to form a stratum having a thickness from the top of the first stratum 35 to the opposite wall of the mold.

4. The method of forming a composite casting composed of a copper alloy free from zinc; and iron, semi-steel or steel, containing manganese, which consists in pouring a 40 quantity of one of the molten metals into the mold to form a lower stratum; partially cooling the lower stratum to a semi-molten state; and then pouring into the mold onto the first stratum a quantity of the other 45 metals to increase the heat of the contiguous copper alloy and to form undulations in the same and to form an upper stratum extending to the upper wall of the mold.

CHAS. T. WILKS.